

## 1

3,232,863

## PROCESS FOR PRODUCING NAPHTHENIC LUBRICATING OILS

William B. Watson, Ponca City, Okla., and Maurice K. Rausch, Chicago Heights, Ill., assignors to Sinclair Research Inc.

No Drawing. Filed Dec. 21, 1961, Ser. No. 161,283  
8 Claims. (Cl. 203—36)

Our invention relates to the production of naphthenic type of lubricating oils. More particularly, our invention relates to the production of naphthenic type lubricating oils from lubricating oil distillate fractions derived from Mid-Continent or mixed base crudes.

Certain crude oils contain a relatively high ratio of naphthenic (cycloalkane) compounds compared with paraffin compounds. Upon proper refining these crude oils yield naphthenic lubricating oils which are particularly desirable for use in grease, diesel engine lubricants and cutting oil formulations. The factors contributing to the particular desirability of naphthenic lubricating oils are their high grease yields, i.e., a high ratio of oil to soap for a given consistency. Further, naphthenic lubricating oils yield soft carbon deposits in diesel engines, particularly in railroad diesels, and consequently cause less wear on moving parts. Naphthenic lubricating oils are highly compatible with the various additives used in cutting oil compositions and for this reason are preferred for such service.

Due to the specific properties possessed by naphthenic lubricating oils the demand for them is very great. Crude oils which yield such lubricating oils, however, are diminishing in supply and from time to time definite shortages of these lubricating oils exist. On the other hand Mid-Continent or mixed base lubricating oil stocks continue to be in large supply.

We have discovered a process whereby these desirable naphthenic type lubricating oils can be derived from the more plentiful Mid-Continent or mixed base lubricating oil stocks.

The process of our invention comprises subjecting a mixed base lubricating oil distillate fraction to solvent extraction by a solvent selective for aromatics in a manner to yield a particular fraction, dewaxing this particular fraction and hydrogenating the dewaxed fraction. Alternatively, the dewaxing step can precede the solvent extraction. The particular fraction is derived by particular treatment of the extract phase of a conventional solvent extraction, rather than from the normally desirable raffinate phase. Such extract phases have few known uses and are unsuitable for use as lubricating oils. Thus, our invention also provides a process for obtaining naphthenic type lubricating oils from a normally undesirable extract phase.

It is desirable to obtain a particular fraction from which most paraffinic and most aromatic components have been excluded. This fraction is obtained by separating the extract phase, from the conventional solvent extraction of a mixed base lubricating oil distillate fraction, into a second extract phase which is similar to the first extract phase in that it has a high aromatic and low paraffin content and a second raffinate phase from which most of the paraffins and aromatics have been

## 2

excluded. It is this second raffinate or heart-cut fraction which is treated by hydrogenation in accordance with the process of our invention. The separation can be carried out by cooling the first extract phase, or by injecting an anti-solvent into the first extract phase or by a combination of cooling and injection of an anti-solvent to produce a second extract and raffinate phase which can then be separated in a settler with the upper (raffinate) phase being the desired or heart-cut fraction. The separation can also be carried out by subjecting the first extract phase to re-extraction by means of a conventional system with a solvent selective for aromatics, using a lower temperature or by adding a solvent containing an anti-solvent or using a combination of a lower temperature and the anti-solvent, to produce the desired raffinate or heart-cut fraction.

Thus, according to the process of our invention a mixed base lubricating oil distillate fraction is subjected to a conventional solvent extraction process to produce an extract phase. The amount of solvent can vary from 100 to 1000 volume percent solvent based upon the lubricating oil fraction. The temperature employed in this extraction process can vary somewhat according to the particular solvent used, e.g., phenol—155 to 210° F.; furfural—150 to 250° F.; liquid sulfur dioxide—less than 150° F. When it is desired to separate this extract phase into second extract and raffinate phases, using the cooling or anti-solvent method described above it is not necessary to remove the solvent prior to further processing of the first extract. Inasmuch as the extract removed from a conventional solvent extraction process will usually be at a temperature about 180° F., it is necessary only to cool the extract to a temperature of about 100 to 125° F. to effect phase separation. While phase separation can be accomplished by the injection of a sufficient quantity of anti-solvent, it is desirable to limit the injection of an anti-solvent, such as water to about 5 to 25 percent by volume. When employing water in this quantity it is preferred to cool the extract to a temperature in the range from about 105 to 135° F. To obtain the second extract and raffinate phases using the re-extraction method described above the quantity of solvent employed in the second extraction step is usually somewhat less than in the first extraction step. Normally it is satisfactory to employ from 50 to 700 volume percent solvent based upon the first extract. As described above, the temperature employed in the re-extraction is usually lower than employed in the first extraction, e.g., phenol—90 to 150° F.; furfural—90 to 200° F. A more specific description of the methods employed in this re-extraction step of our process can be found in U.S. Patent No. 2,943,990.

The extraction steps are operated so that the first extract preferably represents from about 20 to about 70 volume percent of the raw lubricating oil distillate and the second raffinate (the heart-cut) preferably represents from about 20 to 70 volume percent of the first extract. In conducting the extraction steps of the process suitable solvents that can be employed include phenol, furfural, liquid sulfur dioxide, nitrobenzene, nitro paraffins and other solvents selective for aromatics. Such processes and solvents are well known. For example, when employing phenol, a particularly advantageous solvent, the extraction comprises passing a feed stock through a phe-

nol treating tower, removing a raffinate oil from the top of the tower and removing an extract oil from the bottom and removing the phenol from the raffinate oil and extract oil by distillation. A suitable anti-solvent for use in our process is water.

The dewaxing step of the process of our invention can be carried out by employing a conventional lubricating oil dewaxing process such as solvent dewaxing, e.g., with a methyl ethyl ketone and toluene solvent blend, or urea dewaxing through the formation of adducts of urea and straight chain paraffins. The dewaxing can precede the solvent extraction but for the proper control of pour point it is preferred to extract first and then dewax. The extracted and dewaxed fraction is then subjected to catalytic hydrogenation.

The hydrogenation step of our process is conducted at a pressure from about 1000 to about 3500 p.s.i.g., a temperature from about 600 to about 750° F. and at a weight hourly space velocity from about 0.25 to about 3.0 pounds of oil per pound of catalyst per hour. Any of the well known hydrogenation catalysts such as molybdenum, chromium, tungsten, vanadium, platinum, zinc, tin, nickel, copper, iron and cobalt or their oxides or sulfides either unsupported or supported on a suitable catalyst carrier such as alumina or silica can be employed in this step of our process. Particularly advantageous catalysts are the iron transition metals (iron, cobalt and nickel) and the Group VI B metals (chromium, molybdenum and tungsten) especially combinations of metals from each of these groups, for instance, cobalt and molybdenum, nickel and tungsten, and nickel and molybdenum supported on alumina. Of these catalysts we prefer to employ a cobalt-molybdate on alumina catalyst such as that described in U.S. Patent No. 2,898,308.

If it is so desired, the hydrogenated product of our process can be fractionated in order to yield certain narrower fractions particularly suited to certain end uses.

In our process, specific dispersion can be used to control the various steps. Specific dispersion is defined as

$$\frac{n_G^{20} - n_E^{20} \times 10^4}{d_4^{20}}$$

where  $n$ =refractive index and  $d$ =density. Thus, the first solvent extraction preferably should yield an extract having a minimum specific dispersion of 160 and the heart-cut fraction preferably should have a specific dispersion between 135 and 185. Furthermore, the heart-cut fraction should have a gravity of about 15 to 30° API and a viscosity of about 35 to 200 SUS at 210° F. In the hydrogenation step, the specific dispersion of the heart-cut feed should be reduced about 10 to 70, preferably about 20 to 30. Thus, the final hydrogenated product should have a specific dispersion between 105 and 140 depending upon the properties required for end use.

The mixed base lubricating oil distillate fraction is derived from mixed base crude oils which have a composition intermediate that of the paraffinic, e.g., Pennsylvania, and naphthenic types of crude oil. Generally, mixed base crude oil is found in the Mid-Continent area. For example, such crudes include Oklahoma City and East Texas. Inasmuch as the composition of mixed base crude oils is intermediate that of paraffinic and naphthenic crudes the physical properties of a mixed base crude are usually intermediate those of paraffinic and naphthenic crudes. Thus, the fraction of a mixed base crude boiling between 428° F. and 527° F. at atmospheric pressure will have an API gravity between about 33 and 40° API while the fraction boiling between 527° F. and 572° F. at 40 mm. will have an API gravity between about 20 and 30° API and a cloud point above 50° F. The characterization factor of mixed base oils normally falls in the range from 11.5 to 12.1. Mixed base crude oils can

be chemically classified as paraffinic-naphthenic crude oils according to the system set forth in "The Science of Petroleum," volume V, part I, pages 75-77, Oxford University Press, New York, 1953, and A. N. Sachanen, "The Chemical Constituents of Petroleum," pages 419-427, Reinhold Publishing Corporation, New York, 1945. Representative of such crude oils are an Oklahoma City crude with the approximate composition, by weight, of 36% paraffins, 45% naphthenes, 14% aromatics and 5% resins and asphaltenes and a ring analysis showing 65% paraffin side chains, 25% naphthenic rings and 10% aromatic rings and an East Texas crude with the approximate composition of 33% paraffins, 41% naphthenes, 17% aromatics and 9% resins and asphaltenes and a ring analysis showing 60% paraffin side chains, 26% naphthenic rings and 14% aromatic rings. Usually Mid-Continent mixed base crude oils will contain from 60 to 70 percent by weight paraffinic side chains and at least 20 percent by weight naphthenic rings.

To illustrate further the process of our invention reference is made to the following example.

#### Example

25 A mixed base East Texas crude oil was fractionated by atmospheric and vacuum distillation to yield gas, gasoline, kerosene, lube distillate, gas oil and asphalt fractions. The lube distillate fraction had the analysis shown in Table I. This lube distillate was solvent extracted with phenol on a counter-current extraction tower using a solvent dosage of 175 volume percent, a top tower temperature of 191° F., a bottom tower temperature of 178° F., and 3.2 volume percent of water based on solvent injected at the tower bottom. This produced 65.9 volume percent yield of raffinate (Raffinate A) and 34.1 volume percent of extract (Extract B).

Raffinate A was dewaxed using a 50/50 blend of MEK and toluene and a filter temperature of -10° F. to obtain 68.4 volume percent of dewaxed Mid-Continent lubricating oil (Lube C).

Extract B tested 17.3° API gravity, 43.6 SSU at 210° F. viscosity, +60° F. pour, and 194.5 specific dispersion. In order to compare compositions, a portion of Extract B was dewaxed in a manner similar to Raffinate A to yield 45 93.0 volume percent of a finished aromatic oil (Lube D).

A second portion of Extract B was batch solvent extracted with phenol containing 20.0 volume percent water using a solvent dosage of 665 volume percent and a temperature of 105° F. This produced 64.3 volume percent of raffinate (Raffinate E) and 35.7 volume percent of extract (Extract F). Raffinate E was dewaxed in the same manner as Raffinate A to yield 90.2 volume percent of dewaxed lubricating oil (Lube G).

55 Lube G was hydrogenated at 1500 p.s.i.g., 700° F., and 1.0 WHSV over a cobalt-molybdenum supported on alumina, catalyst to yield 98.4 volume percent of finished naphthenic type lubricating oil (Lube H). Lube H represents the product from the process of this invention.

60 Two lubricating oil stocks were prepared by the conventional manner from a blend of equal parts of Gulf Coast Pickett Ridge, Damon and Thompson crude oils. The crude was fractionated by atmospheric and vacuum distillation to yield gas, gasoline, light and medium lubricating oil distillates, gas oil and asphalt. Distillation was over caustic to remove naphthenic acids. The lube distillates were treated with 14 and 25 pounds per barrel of 98% sulfuric acid, respectively, neutralized with caustic and contacted at 180° F. with 3 pounds of fullers earth per barrel of oil. Overall yield from the light lubricating oil distillate (Lube J) was 87.3 volume percent and from the medium lubricating oil distillate (Lube K) 83.5 volume percent. These two lubricating oils are typical of those produced from naphthenic base crude oils.

TABLE I

| Designation                                                        | Raw Lube<br>Dist.<br>Fract. | Lube C                                       | Lube D                                                                           | Lube G                                                                                          | Lube H                                                    | Lube J                                                      | Lube K                                                      |
|--------------------------------------------------------------------|-----------------------------|----------------------------------------------|----------------------------------------------------------------------------------|-------------------------------------------------------------------------------------------------|-----------------------------------------------------------|-------------------------------------------------------------|-------------------------------------------------------------|
|                                                                    |                             | Identity                                     |                                                                                  |                                                                                                 |                                                           |                                                             |                                                             |
|                                                                    |                             | Typical<br>M-Cont.<br>Solv. Re-<br>fined Oil | Dewaxed Ext.<br>from Solvent<br>Refg. Lube<br>Ext. (Lube D)<br>(Aromatic<br>oil) | Dewaxed Raff.<br>from Solv.<br>Refg. Lube<br>Ext. (Lube D)<br>Typ. Feed to<br>Hydrogen.<br>Step | Prod. of Inv.<br>Naph. Oil De-<br>rived from<br>M-C crude | Typical Naph.<br>Lube derived<br>from Naph-<br>thenic Crude | Typical Naph.<br>Lube derived<br>from Naph-<br>thenic Crude |
| <b>Laboratory Tests:</b>                                           |                             |                                              |                                                                                  |                                                                                                 |                                                           |                                                             |                                                             |
| Gravity, °API                                                      | 30.1                        | 33.0                                         | 15.7                                                                             | 21.0                                                                                            | 23.2                                                      | 24.4                                                        | 22.5                                                        |
| Vis. SSU/100° F                                                    |                             | 105.6                                        | 303.8                                                                            | 150.0                                                                                           | 99.89                                                     | 324.3                                                       |                                                             |
| Vis. SSU/210° F                                                    | 38.1                        | 39.9                                         | 45.4                                                                             | 43.7                                                                                            | 41.1                                                      | 37.7                                                        | 48.2                                                        |
| Pour, °F                                                           | +85                         | +10                                          | +5                                                                               | +10                                                                                             | +10                                                       | +5                                                          | +20                                                         |
| Specific Dispersion                                                | 135.0                       | 104.5                                        | 201.6                                                                            | 158.5                                                                                           | 129.6                                                     | 132.8                                                       | 129.9                                                       |
| <b>Hydrocarbon Type Analysis, Weight Per<br/>cent<sup>1</sup>:</b> |                             |                                              |                                                                                  |                                                                                                 |                                                           |                                                             |                                                             |
| Saturates:                                                         |                             |                                              |                                                                                  |                                                                                                 |                                                           |                                                             |                                                             |
| Paraffins                                                          |                             | 21.3                                         | 5.2                                                                              | 9.7                                                                                             | 7.7                                                       | 4.6                                                         | 3.9                                                         |
| Non-Condensed Cycloalkanes                                         |                             | 42.8                                         | 14.2                                                                             | 21.8                                                                                            | 28.2                                                      | 32.8                                                        | 29.6                                                        |
| Condensed Cycloalkanes                                             |                             | 22.3                                         | 9.8                                                                              | 16.6                                                                                            | 22.6                                                      | 24.2                                                        | 27.5                                                        |
| Aromatics—                                                         |                             |                                              |                                                                                  |                                                                                                 |                                                           |                                                             |                                                             |
| Benzenes                                                           |                             | 4.5                                          | 9.6                                                                              | 13.6                                                                                            | 9.6                                                       | 8.8                                                         | 8.1                                                         |
| Indanes, Tetralins                                                 |                             | 3.3                                          | 12.6                                                                             | 9.5                                                                                             | 10.4                                                      | 9.1                                                         | 9.1                                                         |
| Naphthalenes                                                       |                             | 2.5                                          | 6.6                                                                              | 5.6                                                                                             | 5.1                                                       | 5.0                                                         | 5.2                                                         |
| Diphenyls, Acenaphthalenes                                         |                             | 0.6                                          | 8.9                                                                              | 4.9                                                                                             | 4.3                                                       | 4.7                                                         | 4.2                                                         |
| Phenanthrenes, Anthracenes                                         |                             | 0.3                                          | 9.5                                                                              | 3.8                                                                                             | 3.1                                                       | 2.9                                                         | 2.9                                                         |
| Pyrenes, Fluoranthrenes                                            |                             | 0.6                                          | 7.6                                                                              | 3.0                                                                                             | 2.0                                                       | 1.6                                                         | 1.9                                                         |
| Chrysenes                                                          |                             | 0.6                                          | 3.8                                                                              | 1.9                                                                                             | 1.7                                                       | 1.6                                                         | 1.9                                                         |
| Perylenes                                                          |                             | 0.5                                          | 8.2                                                                              | 4.5                                                                                             | 3.3                                                       | 2.9                                                         | 3.5                                                         |
| Polar Compounds                                                    |                             | 0.7                                          | 4.0                                                                              | 5.1                                                                                             | 2.0                                                       | 1.8                                                         | 2.2                                                         |
| Total                                                              |                             | 100.0                                        | 100.0                                                                            | 100.0                                                                                           | 100.0                                                     | 100.0                                                       | 100.0                                                       |

<sup>1</sup> Combination of silica gel chromatography and mass spectrometry.

Table I lists the properties of the various lubricating oils produced in this example. In obtaining the chromatographic data the procedure employed is described in the article, "Properties of High-Boiling Petroleum Products," L. T. Eby, Analytical Chemistry, vol. 25, page 1057, July 1953. The mass spectrometer methods employed are described in "Mass Spectrometric Analysis of High Molecular Weight Saturated Hydrocarbons," R. J. Clerc, Archie Hood and M. J. O'Neal, Jr., Analytical Chemistry, vol. 27, page 868, June 1955, and "Composition of an East Texas Lube Oil Distillate," B. A. Drkin, J. G. Bendoraitis, R. Brown and R. H. Williams, Symposium on Composition of Petroleum Oils, Determination and Evaluation, sponsored by Research Division IV of ASTM Committee D-2, February 8, 9, 1957, New Orleans.

It will be noted that Lube C, which is a typical Mid-Continent solvent refined oil, differs considerably in composition from Lubes J and K, typical naphthenic lubricating oils from South Texas Gulf Coast crude oils. Specifically, Lube C has a considerably higher saturates content and is particularly rich in paraffin.

Lube D, the aromatic extract, on the other hand is high in aromatics and extremely low in cycloalkanes as compared with Lubes J and K.

Lube G, the heart-cut fraction, is more related to Lubes J and K but is still high in aromatic content and low in cycloalkanes.

Lube H, hydrogenated Lube G, represents the product of the process of our invention. It will be noted that Lube H closely approximates the composition of Lubes J and K and has similar properties, with the exception of pour point. However, dewaxing conditions for Lube H can be adjusted, for example by reducing the filtering temperature to -40° F., to yield an oil having pour properties more related to Lubes J and K. More severe dewaxing will also reduce the paraffin content of Lube H. Thus, it can be seen that the process of our invention produces a lubricating oil having a composition and properties similar to those of typical naphthenic lubricating oils and is obtained by the treatment of a mixed base lubricating oil fraction.

We claim:

1. A process for producing naphthenic type lubricating oils having a specific dispersion between about 105 and about 140 from a mixed base lubricating oil distillate fraction which comprises subjecting the mixed base distillate fraction to a solvent extraction treatment including the steps of extracting the distillate fraction with a solvent selective for aromatics to yield a first extract phase comprising about 20 to about 70 volume percent of the mixed base distillate fraction and having a specific dispersion of at least about 160 and separating the first extract phase into a second extract phase and a second raffinate phase from which second raffinate phase most paraffinic and most aromatic components have been excluded by said solvent extraction treatment and said separating and having a specific dispersion of from about 135 to about 185 and comprising about 20 to about 70 volume percent of the first extract phase, subjecting said second raffinate phase to a dewaxing treatment, and hydrogenating the dewaxed second raffinate phase while in contact with a hydrogenation catalyst at a temperature from about 600° F. to about 750° F., a pressure from about 1000 to about 3500 p.s.i.g. and at a weight hourly space velocity from about 0.25 to about 3.0 pounds of the dewaxed second raffinate per pound of catalyst per hour.
2. The process of claim 1 in which the separation of the first extract phase into the second extract and raffinate phases is accomplished by subjecting the first extract phase to at least one of the steps of cooling and injection of an anti-solvent.
3. The process of claim 1 in which the separation of the first extract phase into the second extract and raffinate phases is accomplished by subjecting the first extract phase to re-extraction with a solvent selective for aromatics including at least one of the steps of cooling and injection of an anti-solvent during the re-extraction.
4. A process for producing naphthenic type lubricating oils having a specific dispersion between about 105 and about 140 from a mixed base lubricating oil distillate fraction which comprises solvent extracting the mixed base distillate fraction with a solvent selective for aromatics to yield a first extract phase comprising about 20

to about 70 volume percent of said mixed base distillate fraction and having a specific dispersion of at least about 160, subjecting the first extract phase to re-extraction with a solvent selective for aromatics and containing an anti-solvent at a temperature lower than that at which the first solvent extraction is conducted to yield a second raffinate phase from which most paraffinic and most aromatic components have been excluded by said solvent extraction treatment and said separating and having a specific dispersion of from about 135 to about 185, a gravity from about 15 to about 30° API and a viscosity from about 35 to about 200 SUS at 210° F. and comprising about 20 to about 70 volume percent of said first extract phase, dewaxing the second raffinate phase and hydrogenating the dewaxed second raffinate phase while in contact with a hydrogenation catalyst at a temperature from about 600° F. to about 750° F., a pressure from about 1000 to about 3500 p.s.i.g. and at a weight hourly space velocity from about 0.25 to about 3.0 pounds of the dewaxed raffinate per pound of catalyst per hour.

5. The process of claim 4 in which the hydrogenation

10

5

catalyst consists essentially of an iron transition metal and a group VI B metal supported on alumina.

6. The process of claim 4 in which the hydrogenation catalyst is a cobalt-molybdate supported on alumina catalyst.

7. The process of claim 1 in which the hydrogenation catalyst consists essentially of an iron transition metal and a group VI B metal supported on alumina.

8. The process of claim 7 in which the hydrogenation catalyst consist essentially of a cobalt-molybdate supported on alumina.

References Cited by the Examiner

UNITED STATES PATENTS

|    |           |        |                |        |
|----|-----------|--------|----------------|--------|
| 15 | 2,248,373 | 7/1946 | Merrill et al. | 208-36 |
|    | 2,780,581 | 2/1957 | Macke et al.   | 208-36 |
|    | 2,943,990 | 7/1960 | Rausch et al.  | 208-36 |
|    | 2,967,144 | 1/1961 | Cole           | 208-87 |
|    | 2,967,147 | 1/1961 | Cole           | 208-87 |
|    | 2,984,616 | 5/1961 | Burke et al.   | 208-87 |

DELBERT E. GANTZ, Primary Examiner.

ALPHONSO D. SULLIVAN, Examiner.